

## UNITED STATES PATENT OFFICE

2,408,668

## ELECTROLYSIS OF COPPER

William Clark Mason, Inspiration, Ariz., assignor  
to Inspiration Consolidated Copper Company,  
a corporation of Maine

No Drawing. Application May 27, 1943,  
Serial No. 488,745

1 Claim. (Cl. 204—108)

1

This invention relates to electrolytic precipitation of metal, more particularly to the precipitation of copper from sulphuric acid electrolytes, and has for its object the provision of an improved method of controlling cathode sprouts. The wart-like growths called "sprouts," which form on cathodes as the metal is deposited, reduce the electrical efficiency and frequently become so large as to cause short circuits. The invention provides a simple and effective method for inhibiting the growth of sprouts on copper cathodes with a resulting increase in the electrical efficiency.

In the electrolytic precipitation of copper as practiced heretofore, the sprouts form as needle-like or tree-like growths on the surfaces of the copper cathodes during the electrolytic deposition. These sprouts grow to such length that they may touch the anode, thus causing a short circuit.

I have discovered that an excess of concentrated sulphuric acid treated with a petroleum oil of naphthenic origin, such as California petroleum, has the property of inhibiting the growth of copper sprouts when the oil-treated acid is suitably incorporated in the electrolyte. In accordance with my invention, the concentrated sulphuric acid is treated with the petroleum, either crude or a distillation product, such as fuel oil, Diesel oil and the like, and a product of the reaction remains in the acid as the beneficial constituent which is added to the electrolyte along with the acid.

The oil-treated acid may be incorporated in the electrolyte in any suitable manner; for example, it may be added from time to time throughout the day to the electrolyte, to the plant supply of acid, or to the make-up acid which is used to replenish the acid losses.

In preparing the oil-treated acid, the California petroleum is agitated with strong sulphuric acid, for example, 78% to 95% acid, with the formation of water soluble and acid soluble products which remain in the acid, and an oily or sludge-like residue which separates on standing. In addition to the water and acid soluble products remaining in the acid, the acid contains materials in suspension, such as tars, which have not been completely identified. In using a fuel oil of about 16° gravity, about one part of oil is agitated with an excess of strong sulphuric acid, for example, one volume of oil to five volumes of acid, and the mixture is allowed to stand for several hours or until a heavy tar-like residue comes to the top and is discarded. Diesel oil may be used with an

2

excess of strong sulphuric acid, for example, in amounts of about one volume of oil to from one to two and one-half volumes of acid. In using Diesel oil, however, a colorless oil comes to the top which may be recovered and used as a fuel.

In carrying out a method of the invention I may add continuously a small amount of oil-treated acid to the electrolyte as it enters the electrolytic plant. The quantity of this oil-treated acid should be about that of the acid necessary to treat the volume of oil required. The volume of oil required varies with the appearance of the copper deposit, and to a large extent varies with the amount of copper precipitated.

In operations involving the leaching of ore, it is more convenient to add the oil-treated acid to the larger volume of new acid required as this new acid has to be more or less uniformly added to the electrolyte. In such operations, it has been found that 1.4 gallons to 2.8 gallons of oil have to be treated with an excess of acid for every ton of copper precipitated, the oil-treated acid containing the beneficial substance removed from the oil being incorporated in the electrolyte.

The quantity of oil to be treated with an excess of acid, necessary to yield an oil-treated acid to satisfy electrolyte requirements as to retarding sprout growth, may be expressed in the following manner: In an operation, for example, where about 2400 gallons of electrolyte flows to the electrolytic plant every minute, about 0.04 to 0.09 gallon of oil are treated for every 1000 gallons flowing to the electrolytic plant.

The following illustrate specific examples:

*Example I*

40 One volume of California fuel oil of about 16° gravity was agitated with five volumes of strong sulphuric acid for about one hour. After agitating, the mixture was allowed to stand for several hours. After standing, the heavy tar-like residue on top was skimmed off and discarded. The remaining liquid, which is the oil-treated acid, was then added to an electrolyte flowing to a set of electrolytic cells in the proportion of one gallon of oil-treated acid to about sixty gallons of plant acid. The growth of sprouts, and the electrode efficiencies of this set of cells were then compared to a duplicate set of cells using the same type of electrolyte but not having any of 55 the above mixture added.

The average results of several such tests show the following results.

|                                                      | No oil-treated acid in electrolyte | Oil-treated acid in electrolyte |
|------------------------------------------------------|------------------------------------|---------------------------------|
| Cathode efficiency.....percent.....                  | 69.2                               | 71.9                            |
| Difference.....do.....                               |                                    | +2.7                            |
| Anode efficiency.....percent.....                    | 72.6                               | 73.9                            |
| Difference.....do.....                               |                                    | +1.3                            |
| Sprouts removed from cathode surfaces.....grams..... | 121                                | 24                              |
| Difference.....per cent.....                         |                                    | -80                             |

*Example II*

One volume of California Diesel oil was agitated with  $2\frac{1}{2}$  volumes of strong sulphuric acid for about  $1\frac{1}{2}$  hours. After agitation, the mixture was allowed to stand for about one hour. A clear oil came to the top and was decanted away from the acid residue. The oil-treated acid containing its dissolved beneficial constituents was then added to the electrolyte in proportions similar to those of Example I. This electrolyte was then run through the electrolytic cells and the results of such cells were compared with the results of like cells using an untreated electrolyte. The following average results obtained were from several tests:

|                                                      | No oil-treated acid in electrolyte | Oil-treated acid in electrolyte |
|------------------------------------------------------|------------------------------------|---------------------------------|
| Cathode efficiency.....percent.....                  | 64.8                               | 66.7                            |
| Difference.....do.....                               |                                    | +1.9                            |
| Anode efficiency.....per cent.....                   | 61.6                               | 63.1                            |
| Difference.....do.....                               |                                    | +1.5                            |
| Sprouts removed from cathode surfaces.....grams..... | 191                                | 19                              |
| Difference.....per cent.....                         |                                    | -90                             |

It can be seen from the above examples that

when small quantities of oil-treated acid containing organic reaction products produced in the treatment of California petroleum fractions by strong sulphuric acid are added to an electrolyte, the quantity of sprouts is greatly reduced. The improvements in the various electrode efficiencies are due to the elimination of sprouts on the cathodes.

The cathode efficiency referred to herein means the amount of copper actually deposited, divided by the amount of copper that theoretically should have been deposited for the quantity of electric current that passed through the electrolyte. When this result is multiplied by 100, the answer is in percent.

The anode efficiency referred to herein means the amount of ferrous iron oxidized to ferric iron at the surface of the anode, divided by the amount of ferrous iron that theoretically should have been oxidized for the amount of copper precipitated out on the cathode. When this result is multiplied by 100, the answer is percent anode efficiency.

I claim:

In a process for the production of electrolytic copper cathodes involving electrolytic precipitation of copper from a sulphuric-acid-containing electrolyte, the improvement which comprises inhibiting the formation of sprouts on the cathodes during electrolysis by adding to the electrolyte an oil-treated acid obtained by agitating one volume of naphthenic crude oil with about five volumes of about 78% to 95% sulphuric acid, causing the oil-treated acid to settle and a tar-like material to form on top, and removing the tar-like material, the resulting oil-treated acid being added to the electrolyte in an amount corresponding to that produced by the treatment of about 1.4 to 2.8 gallons of the crude oil per ton of copper cathodes precipitated.

W. CLARK MASON.